

Patented Oct. 13, 1931

1,827,204

## UNITED STATES PATENT OFFICE

SUMNER REDWAY MASON, OF WILMETTE, ILLINOIS, ASSIGNOR TO WESTERN ELECTRIC COMPANY, INCORPORATED, OF NEW YORK, N. Y., A CORPORATION OF NEW YORK

### METHOD OF PROTECTING METAL SURFACES

No Drawing.

Application filed October 18, 1927. Serial No. 227,061.

This invention relates to a method of protecting metal surfaces and is related to my copending application, Serial No. 227,060, filed October 18, 1927.

5 The object of the invention is to provide a simple, effective and economical method of rendering metal surfaces capable of resisting the action of moisture or other influences tending to corrode such surfaces.

10 In accordance with the general features of the invention, an article having a metal surface which it is desired to protect is connected as a cathode in an electrolytic cell in which the bath employed contains a salt of an acid containing chromium, such as sodium chromate or potassium dichromate, as an electrolyte. An initial electric current of sufficiently low cathode current density to insure substantially no metallic chromium deposition 15 is passed through the cell for a short period of time after which the article is removed from the cell and dried. If desired, the surface of the article which has been subjected to the above described treatment may 20 be readily coated with a protective paint, such as a japan, in order to give additional protection and to give the surface a desired finish.

It has been found by experiment that when such metals as iron, zinc, cadmium, copper, 25 silver, etc. are connected as cathodes in an electrolytic cell in which the bath contains a salt of an acid containing chromium, such as sodium chromate or potassium dichromate, and when a current of sufficiently low cathode current density to provide conditions under 30 which metallic chromium is not deposited, is passed through the cell for a short period of time the surfaces of the articles are rendered passive to the extent that they will resist the 35 corrosive action of atmospheric agents for a much longer period of time than surfaces which have not been so treated. The surfaces rendered passive are also quite resistant to the action of sulphur, acids, such as 40 nitric acid and hydrogen sulphide, and numerous other corrosive substances even after the treated articles have been subjected to abrasion. This phenomenon provides a very 45 effective method for protecting metal sur-

faces and it constitutes the subject matter of the present invention.

Although it is to be understood that the method of protecting metal surfaces forming the subject matter of this invention is applicable to numerous metals and that the ingredients and conditions under which the method is practiced may be varied within a wide range, a few specific embodiments of the invention will be described in detail in order 55 to enable persons skilled in the art to practice the invention.

One embodiment of the invention consists in a method for protecting the surfaces of articles made of iron. In this embodiment of 60 the invention an electrolytic cell is employed in which the bath comprises a water solution containing 31 grams per liter of sodium chromate in which is connected an anode of any suitable insoluble material, such as iron, 65 platinum or lead. The article to be treated is connected as a cathode in the above described electrolytic cell, an electric current of a cathode current density of 50 to 100 amperes per square foot is passed through the cell for a 70 short period of time, and the temperature of the bath is maintained at room temperature 75 (20-25° C.) during the passage of the current. For rendering the surfaces resistant to the action of atmospheric agents 5 to 15 80 minutes has proven to be a satisfactory length of time for the electrolytic treatment. After this treatment the article is removed from the electrolytic cell and dried in any suitable manner. An iron article so treated will be found 85 to have a greatly increased resistance to atmospheric corrosion and will not rust to any great extent unless exposed to extreme conditions for a long period of time.

Another very practical use to which the 90 process may be put is in the protection of articles coated with other metals such as zinc or cadmium. It has been attempted heretofore in some instances to coat articles, which it is desired to protect, with a coating of 95 zinc, since zinc is resistant to corrosive agents, and then to apply a coating of a protective paint, such as a japan, upon the zinc coating. It has been found, however, that the zinc in the first coating has a tendency to react with 100

the oleagenous fatty acids, such as oleic or palmitic acid, present in the protective paint to form zinc soaps which will prevent the adherence of the protective paint to the zinc coating with the result that the protective paint has a tendency to scale off of the zinc coating after a short period of time.

In this embodiment of the invention, the article to be protected is first coated with another metal such as zinc or cadmium and the coated article is then connected as a cathode in an electrolytic cell of the type described above in which the bath comprises a water solution containing 65 grams per liter of potassium dichromate and an electric current of low cathode current density is passed through the cell for a short period of time while the bath is maintained at room temperature. The article is then removed from the electrolytic cell and dried. It will be found that after such treatment the metallic coating upon the article has been rendered passive in the same manner as the iron article hereinbefore described, and an article so treated will offer great resistance to corrosion. If desired, the article treated in the manner just described may be coated with a protective paint, such as a japan, in order to give additional protection to the article and to provide a desired finish. When the article is protected in this manner the surface of the zinc or cadmium which has been subjected to the above outlined treatment does not react with the fatty acids in the paint to form metallic soaps and as a consequence the paint adheres firmly to the zinc coating even when subjected to very adverse conditions.

It is believed that the embodiments of the invention just described will sufficiently illustrate how the invention may be practiced, but it is, of course, to be understood that the invention is not limited to the specific examples given hereinbefore. The invention may be practiced with satisfactory results upon metals other than iron, zinc and cadmium, such as copper and silver, and also the conditions under which the articles are rendered passive may be varied within a wide range. For example, the bath included in the electrolytic cell need not necessarily be composed of a water solution containing 31 grams per liter of sodium chromate or 65 grams per liter of potassium dichromate, but the amounts of these ingredients present in the baths may be varied within wide limits and still satisfactory results may be obtained. Nor does the bath need to contain only sodium chromate or potassium dichromate in water solution, but additional conducting materials may be present in order to vary the operating conditions of the bath. Satisfactory results may also be obtained when other alkali salts of chromic or dichromic acids are employed and such materials as potassium, ammonium and lithium chromates and

sodium, ammonium and lithium dichromates may be substituted for the above described materials in order to render metal surfaces resistant to corrosive agents. Also the amount of current flowing through the cell may be varied over a wide range so long as the initial cathode current density is maintained below the range within which metallic chromium would be deposited from the particular bath used in quantities more than 70 traces. The temperature of the bath may also be varied to provide the optimum conditions of operation obtainable with the particular bath and current density employed, and also the time of treatment may be varied. 75 Satisfactory results may be usually obtained, however, when the bath is operated at room temperature (20 to 25° C.) and the article is treated for from three to fifteen minutes in the electrolytic cell. 80

A satisfactory theory of the reactions which take place during the above described operations has not yet been developed, but some or all of a number of changes may occur. For example, the surface of the metal 90 which it is desired to protect may be oxidized or otherwise chemically changed. Or a physical change or displacement may be effected in the molecules comprising the surface layers of the metal, so that the surface 95 of the metal is rendered passive. Or it may be possible that the metal surface is coated with an extremely thin film composed of a compound or compounds derived from the electrolytic bath. Whatever the changes or 100 reactions which occur may be, a treatment embodying the invention renders the surface of the treated metal resistant to corrosion, and at the same time the weight and dimensions of the treated article remain substantially unchanged. Also the appearance 105 of the article remains practically unchanged in most instances after treatment. For example, copper articles originally having bright, clean surfaces usually exhibit a similar appearance with possibly a slight iridescence being noticeable after having been treated in accordance with the invention, but there is no evidence that the articles are coated with any colored or colloidal material of 110 the types sometimes found in electroplating baths for the deposition of metallic chromium. 115

The method described above provides an extremely simple and inexpensive means 120 whereby surfaces of metal articles may be protected against corrosion and abrasion without any material variation in the weight or dimensions of the article. The treatment is especially effective in treating irregular 125 shaped articles for not only the plane surfaces of the articles are protected, but the protective effects are also obtained in corners, crevices, and the walls of holes in the articles. 130

By the statement employed hereinbefore in the specification and also in the appended claims, that the cathode current density is maintained at a value below those in the range within which metallic chromium is deposited is meant a cathode current density of such value that no more than traces of metallic chromium are deposited. The word "paint" as used herein in the specification and claims is intended to include japsans, lacquers, varnishes, paints and other similar protective substances.

What is claimed is:

1. A process for protecting surfaces of metal articles, which consists in subjecting an article as a cathode in a bath containing 65 grams of potassium dichromate per liter to an electric current of a cathode current density below the range in which chromium is deposited for from 5 to 15 minutes and maintaining the bath at room temperature. 85
2. A process for protecting surfaces of metal articles, which consists in coating the surface of an article with a metal of the zinc group and subjecting the article as a cathode in a bath including a salt containing chromium to an electric current of a cathode current density below the range within which chromium is deposited, and coating the treated article with a protective paint. 90
3. A process for protecting surfaces of metal articles, which consists in coating the surface of a metal article with zinc, subjecting the coated article as a cathode in a bath including an alkali salt of an acid containing chromium to an electric current of a cathode current density below the range within which chromium is deposited, and coating the treated article with a protective paint. 95
4. A process for protecting surfaces of metal articles, which consists in coating the surface of an article with another metal, subjecting the coated article as a cathode in a bath containing a dichromate to an electric current of a cathode current density below the range within which chromium is deposited, and coating the treated article with a protective paint. 100
5. A process for protecting surfaces of metal articles, which consists in coating the surfaces of an article with zinc, subjecting the article as a cathode in a bath containing 65 grams of potassium dichromate per liter to an electric current of a cathode current density below the range within which chromium is deposited for from 5 to 15 minutes, maintaining the bath at room temperature, removing the article from the bath, drying the article and coating the treated article with a protective paint. 115
6. A process for protecting surfaces of metal articles which consists in subjecting the article as a cathode in a bath containing about 65 grams of potassium dichromate per liter to an electric current of a cathode cur-

rent density below the range in which chromium is deposited.

7. A process for protecting surfaces of metal articles which consists in coating the surface of an article with zinc, subjecting the article as a cathode in a bath containing about 65 grams of potassium dichromate per liter to an electric current of a cathode current density below the range in which chromium is deposited, and covering the thus treated article with a protective paint. 75

In witness whereof, I hereunto subscribe my name this 30th day of September, A. D. 1927.

SUMNER REDWAY MASON. 80

85

90

95

100

105

110

115

120

125

130